

## UNITED STATES PATENT OFFICE

2,079,228

UNSATURATED ESTERS AND SULPHATES  
THEREOF

Walther Schrauth, Berlin-Dahlem, Germany,  
assignor, by mesne assignments, to "Unichem"  
Chemikalien Handels A.-G., Zurich, Switzerland,  
a corporation of Switzerland

No Drawing. Application July 18, 1932, Serial  
No. 623,298. In Germany July 17, 1931

4 Claims. (Cl. 260—99.12)

(Granted under the provisions of sec. 14 act of  
March 2, 1927; 357 O. G. 5)

It is well-known that by conversion of technical oil and fatty acids with low-molecular alcohols, such as methyl-, ethyl-, and isopropyl-alcohol, artificial fatty acid esters are arrived at which owing to their thin liquid and fatty characteristics represent valuable assistants in the textile industry (cf. German Patent No. 388,219).

It has been found that in treating textile fibres and fabrics, some kinds of leather and other similar materials definite particular effects can be achieved, such as could only previously be achieved by the use of natural neat's-foot oil if, instead of using the latter use is made of the esters of unsaturated mono-basic fatty acids with high-molecular univalent saturated or unsaturated fatty alcohols with at least 8 carbon atoms. These esters which, for instance, can be obtained by heating suitable fatty acids with the alcohols mentioned with or without catalysts but which are also contained in natural products, have a more or less low coagulation point according to their composition, so that they can be adjusted to suit all technical requirements in use. They can be used as they are or else in a sulphated condition, as mentioned above, in the first place for greasing leather, but also for treating animal or vegetable fibres and fabrics. Goods treated become soft and pliable, and leather greased with these esters loses its brittleness and tendency to crack.

The technical advantage of this in comparison with natural neat's-foot oil which always has the same chemical composition, lies in the fact that one can combine the fatty acid with the fatty alcohol in any manner desired and so obtain esters possessing considerably more suitable properties than natural neat's-foot oil. The greasing value is therefore in numerous cases greater. Further, whilst esters formed from lower molecular alcohols possess an unpleasant, spirity smell or a typically penetrating ester smell which makes it more difficult to work with such products, the esters here in question are practically odorless.

Example I

282 kilos of oleic acid are esterified in the presence of 15 kilos of concentrated sulphuric acid with 158 kilos of decyl alcohol at about 80-100°

C. A surplus of fatty alcohol is recommendable as it has a favorable effect on the yield, and on completion of the esterification and if desired, after washing with water, it can be steamed off in a vacuum.

The ester prepared in the described manner facilitates considerably the weaving of wool, cotton and other fibres and it can also be used to assist in the tearing process in the manufacture of artificial wool. It is recommended that about 4-5% of the ester be used for fibres worked according to the carded yarn process, and about 1% for those worked on the worsted systems.

Example II

282 kilos of phytetoleic acid are esterified with 260 kilos of oleyl alcohol. After it has been worked up the ester obtained is sulphated with 140 kilos of concentrated sulphuric acid at 25-30° C., washed with cooking salt or Glauber's salts solution and neutralized in any way desired.

A sulphated product results which, in a 2-3% solution in water meets the requirements of the leather industry for a leather greaser which resists cold and does not effloresce, and it obtains better softening effects than are obtained with sulphonated natural neat's-foot oil which has been treated by the freezing process.

What I claim is:

1. An oil for treating fibrous material which consists principally of esters of phytetoleic acid and oleyl alcohol.

2. An oil for treating fibrous material which consists principally of sulphated esters of phytetoleic acid and alcohol of the group consisting of the unsaturated aliphatic mono-hydric alcohols having 8 or more carbon atoms in the molecule.

3. An oil for treating fibrous materials which consists principally of sulphated esters of phytetoleic acid and oleyl alcohol.

4. An oil for greasing fibrous materials which consists principally of a material selected from the group consisting of the esters of phytetoleic acid and aliphatic straight chain mono-hydric alcohols having 8 or more carbon atoms in the molecule, and the sulphates of these esters.

WALTHER SCHRAUTH.